

Jan. 1, 1929.

1,697,233

E. FISCHER

DISTANT COMMUNICATION CABLE

Filed Jan. 13, 1927

Fig. 1



Fig. 2



Fig. 3



Fig. 4



Inventor:

Ernst Fischer

by *Heer'gut Bux.*  
*mit akt'go.*

## UNITED STATES PATENT OFFICE.

ERNST FISCHER, OF BERLIN-TEMPELHOF, GERMANY, ASSIGNOR TO SIEMENS-SCHUCKERTWERKE GESELLSCHAFT MIT BESCHRÄNKTER HAFTUNG, OF BERLIN-SIEMENS-STADT, GERMANY, A CORPORATION OF GERMANY.

## DISTANT-COMMUNICATION CABLE.

Application filed January 13, 1927, Serial No. 160,950, and in Germany October 6, 1925.

My invention relates to distant communication cables with a constant distributed self inductance.

In cables of this type the copper conductor is covered or enveloped with a ribbon or wire of magnetic material for the purpose of increasing the inductivity. In order to secure a good effect this magnetic material should have as high a degree of permeability as possible. It is, however, known that the permeability of such materials is reduced, if they are subjected to a tensile stress, even a slight one. In the annealing process necessary in the manufacture of cables after winding the magnetic material upon the copper conductor considerable stresses are set up in the magnetic material wound upon the conductor owing to the different coefficients of expansion of the copper and the magnetic material, usually steel or iron, so that the permeability of the magnetic material is considerably reduced and its magnetic properties suffer thereby.

This drawback is eliminated by my invention according to which the magnetic material is wound upon the conductor as a corrugated or otherwise suitably shaped tape or wire. When employing such a ribbon or wire the tensile stress set up during the annealing processes owing to the greater expansion of the copper conductor will only cause a slight straightening out or reduction of the amplitude of the corrugations or waves of the material without the material itself being subjected to any tensile stress. As it is difficult to wind corrugated ribbon or wire into a reel and to unwind it again, a smooth ribbon or wire is preferably passed through a corrugating device on its way to the copper conductor, so that the shape desired is only imparted to the material immediately before its application to the copper conductor.

I have illustrated my invention in the accompanying drawings in which Fig. 1 illustrates a corrugating device for the material.

Fig. 2 illustrates a corrugated ribbon applied helically to the cable conductor.

Fig. 3 illustrates a corrugated wire helically applied to the cable conductor.

Fig. 4 shows the conductor covered with a corrugated ribbon being drawn through a compressing die.

It has been found to be advantageous to provide the material with excessively high corrugations or the like when it is wound on the conductor, and to reduce the height of these corrugations when the material thus applied is in position, by passing the cable with the corrugated material through a tapering die, such as is shown at 10 in Fig. 4. This flattens out any prominent portions of the wrapping as shown at 12, and reduces the outer diameter of the wrapping to uniform size as shown at 11 in Fig. 4. In this way very uniform corrugations are obtained in the magnetic covering.

The magnetic material may of course, be bent into other suitable shapes than simple corrugations, for instance into U-shape, so long as no stressing of the material but only a change in its shape takes place when the conductor around which it is wrapped expands. It will be understood that in this case also it is advantageous to start with a straight ribbon or wire and only to bend it into the U-shape immediately before its application to the conductor, by passing it through a suitable device.

Various modifications and changes may be made without departing from the spirit and the scope of the invention, and I desire, therefore, that only such limitations shall be placed thereon as are imposed by the prior art.

I claim as my invention:—

1. In a line cable having a constant distributed self inductance, a covering for the conductor consisting of a corrugated ribbon of magnetic material of high permeability.

2. In a line cable having a constant distributed self inductance, a covering wound on the conductor and consisting of corrugated magnetic material of high permeability.

3. In the method of making a line cable having a constant distributed self inductance, the passing of a straight length of magnetic material of high permeability through a corrugating device and applying the corrugated

material helically to the conductor as it leaves the corrugating device.

4. In the method of making a line cable having a constant distributed self inductance, the passing of a straight length of magnetic material of high permeability through a corrugating device and applying the corrugated material helically to the conductor as it leaves

the corrugating device and drawing the covered conductor through a compressing die. 10

5. As a new article of manufacture, a line cable comprising a conductor having a helically applied iron corrugated ribbon.

In testimony whereof I affix my signature.

ERNST FISCHER.